

1

3,403,504  
**STRETCHABLE TEXTILES PRODUCED FROM THE BACK-TWISTING OF HIGHLY SWOLLEN CELLULOUS YARNS**  
Carl Hamalainen, Metairie, Hubert H. St. Mard, New Orleans, and Albert S. Cooper, Jr., Metairie, La., assignors to the United States of America as represented by the Secretary of Agriculture  
No Drawing. Filed July 13, 1966, Ser. No. 564,735  
5 Claims. (Cl. 57—164)

## ABSTRACT OF THE DISCLOSURE

A process which involves swelling cellulosic yarns either slack or under tension, both of normal and of high twist construction; washing and drying the yarns, to set the configuration; and backtwisting the yarns thereby producing stretch yarns which may be woven to produce fabrics with excellent stretch properties.

A non-exclusive, irrevocable, royalty-free license in the invention herein described, throughout the world for all purposes of the United States Government, with the power to grant sublicenses for such purposes, is hereby granted to the Government of the United States of America.

This invention relates to the production of stretch textile material by swelling either slack or under tension cellulosic yarns of normal- and high-twist construction followed by backtwisting to produce stretch yarns and then weaving the resultant yarns into fabric to produce fabric with stretch properties.

Most stretch cotton fabrics are going into apparel—slacks, blouses, pajamas, uniforms for waitresses and nurses, and other garments—but upholstery and slipcover fabrics are also being made. Stretch adds comfort and allows the fabric to “give” at knees and elbows without unsightly bagging.

Stretch yarns have been produced by treating highly twisted yarns with crosslinking agents, heat curing them in this highly twisted state and then backtwisting beyond the neutral ply twist. Stretch has also been obtained by shrinking the yarn about 40 to 70% by tensionless mercerization followed by subsequent washing and drying without restretching the yarn. Highly chemically modified yarns, such as acetylated yarns, have been heat set followed by twisting techniques to produce stretch. This results from the deformation of the yarns which are thermoplastic and maintaining the deformed structure after twisting. Yarns which have been grafted with a polymer followed by backtwisting or false-twisting results in stretch properties without heat-setting since the grafting tends to fix or set the yarn. This is demonstrated in our copending application Ser. No. 564,759 filed of even date, entitled “Cotton Stretch Yarn by Graft Polymerization of Vinyl Monomers Followed by Backtwisting or False-twisting.”

Tensionless mercerization procedures produce stretch in yarn by virtue of its shrinkage effects. This is the basis for the slack mercerizing process for producing stretch.

2

Mercerization causes a great deal of swelling in cellulosic fibers with concomitant disruption of hydrogen bonds. These bonds are reestablished in new positions after swelling, washing, and drying procedures. Disrupting the geometry of these highly swollen yarns as by backtwisting, results in a coiled or crimped structure with stretch properties.

For the practice of this invention, various conditions for swelling may be employed. Swelling may be carried out slack without any tension or it may be carried out with sufficient tension to prevent any shrinkage of the yarns being treated, or it can be swollen with a greater amount of tension to stretch the yarns during treatment. In this practice of the invention, we have retained the original length of the yarn skeins during swelling under tension. Swelling may be carried out in any caustic solution of suitable strength. We prefer the use of caustic solution of about 23% sodium hydroxide. A wetting agent, such as 1% Dypenol, is generally employed, although any other suitable wetting agent may be used and the swelling can also be effected without a wetting agent. An added swelling agent, such as sodium thiocyanate, may be used to enhance the swelling of the cellulose in the caustic.

Although any temperature in which effective swelling may be accomplished can be used, in the practice of the present invention we chose ambient room temperature of about 25° C. and an elevated temperature of about 92° C.

In the practice of the present invention, the highly swollen yarns were prepared from scoured and bleached 24/2 cotton yarn, the normal singles twist being 4TM-Z, and the ply twist 4TM-S. The high-twist yarn had 4TM-Z single twist and 7TM-Z ply twist construction. This does not preclude that other twist multiples or constructions could not be used. Other cellulosic fibers of synthetic or natural origin such as rayon, high wet modulus rayon, linen, ramie, jute, hemp, sisal, and the like may be used. Also blends and mixtures of the above fibers may be included. Blends with hydrophobic synthetic fibers also are suitable if a sufficient amount of cellulosic fibers are used to effect adequate swelling.

In general the invention can be described as a process for imparting improved stretch properties to cellulosic textiles comprising:

(a) Wetting a cellulosic yarn of normal-twist construction, while said yarn is under no tension, with an aqueous solution containing about 23% by weight of sodium hydroxide and about 1% by weight of a wetting agent compatible with the said 23% sodium hydroxide solution, at about from 25° to 92° C. for periods of time about from 15 to 60 minutes;

(b) Washing, drying, scouring, and washing and drying in the ordinary manner;

(c) Back-twisting the treated yarn; and

(d) Allowing the back-twisted yarn to relax in water.

The process can be varied to include yarns of high-twist construction and/or while varying the tension during the wetting step (a).

In order that the concept of the invention may be more fully understood, the following examples are set forth primarily for the purpose of illustration and any specific enumeration of detail contained therein should

not be interpreted as a limitation of the case, except as indicated in the appended claims.

## EXAMPLE 1

Bleached and scoured 24/2 normal-twist cotton yarns of 4TM-Z singles and 4TM-S ply twist construction were skeined into 500 yard skeins. Six 500-yard skeins were treated in 23% sodium hydroxide solution containing 1% Dypenol wetting agent under each of the conditions listed for mercerization. The single fiber properties (as obtained on the Uster Automatic Single Yarn Tester) of the unrelaxed yarns after they had been washed, dried, and backtwisted 8TM in the Z direction are shown in Table 1.

TABLE 1

|    | Mercerizing conditions               | Breaking load, Gm. | Elongation, percent | Tex. No. |
|----|--------------------------------------|--------------------|---------------------|----------|
| 5  | Tension, 25° C., 15 min.             | 702                | 11.1                | 56.3     |
|    | Slack, 25° C., 15 min.               | 817                | 22.3                | 67.5     |
|    | Tension, 92° C., 60 min.             | 682                | 10.5                | 55.6     |
|    | Slack, 92° C., 60 min.               | 759                | 19.6                | 60.8     |
|    | Tension, 92° C., 60 min., NaSCN (7%) | 690                | 11.3                | 58.8     |
|    | Slack, 92° C., 60 min., NaSCN (7%)   | 787                | 19.0                | 66.3     |
| 10 | Untreated control                    | 660                | 7.6                 | 48.1     |

There is an improvement in elongation and breaking strength in the unrelaxed single yarn.

TABLE 2

| Mercerizing conditions               | 1 inch strip |                 | 2 inch strip, 5 cycles, 2-lb. load |                 | Recovery 24 hr., percent |
|--------------------------------------|--------------|-----------------|------------------------------------|-----------------|--------------------------|
|                                      | B.S., lbs.   | Elong., percent | Stretch, percent                   | Growth, percent |                          |
|                                      |              |                 | 1 min.                             | 24 hr.          |                          |
| Tension, 25° C., 15 min.             | 50.4         | 110             | 62                                 | 13.8            | 10.0                     |
| Slack, 25° C., 15 min.               | 58.3         | 132             | 63                                 | 16.0            | 12.2                     |
| Tension, 92° C., 60 min.             | 46.8         | 112             | 65                                 | 16.6            | 12.6                     |
| Slack, 92° C., 60 min.               | 54.5         | 129             | 62                                 | 16.4            | 13.0                     |
| Tension, 92° C., 60 min., NaSCN (7%) | 47.8         | 111             | 66                                 | 16.4            | 12.7                     |
| Slack, 92° C., 60 min., NaSCN (7%)   | 55.0         | 129             | 65                                 | 16.8            | 13.1                     |
| Untreated control                    | 51.5         | 22              | 10                                 | 1.4             | 1.1                      |

## EXAMPLE 2

30

The yarns prepared in Example 1 were woven into fabric using them as filling yarns only with 40 picks per inch filling. The fabric was relaxed in hot water and dried. The stretch properties of these fabrics are shown in Table 2. There is a considerable increase in the amount of elongation at break of the one-inch strip fabric and excellent stretch and recovery of the two-inch strips after 5 cyclic loadings with 2-lb. load.

## EXAMPLE 3

40

Bleached and scoured 24/2 high twist cotton yarn of 4TM-Z, singles and 7TM-Z ply twist construction were skeined into 500 yard skeins. Six-500 yard skeins were

TABLE 3

|    | Mercerizing conditions               | Breaking load, gm. | Elongation, percent | Tex. No. |
|----|--------------------------------------|--------------------|---------------------|----------|
| 35 | Tension, 25° C., 15 min.             | 636                | 7.8                 | 48.3     |
|    | Slack, 25° C., 15 min.               | 665                | 9.3                 | 50.1     |
|    | Tension, 92° C., 60 min.             | 615                | 8.0                 | 48.4     |
|    | Slack, 92° C., 60 min.               | 630                | 10.6                | 49.3     |
|    | Tension, 92° C., 60 min., NaSCN (7%) | 630                | 8.0                 | 48.1     |
|    | Slack, 92° C., 60 min., NaSCN (7%)   | 647                | 9.5                 | 52.1     |
| 40 | Untreated control                    | 660                | 7.6                 | 48.1     |

The elongation and strength of the high-twist yarns after backtwisting was not as high as that of the normal-twist yarn.

TABLE 4

| Mercerizing conditions               | 1 inch strip |                 | 2 inch strip, 5 cycles, 2-lb. load |                 | Recovery 24 hr., percent |
|--------------------------------------|--------------|-----------------|------------------------------------|-----------------|--------------------------|
|                                      | B.S., lb.    | Elong., percent | Stretch, percent                   | Growth, percent |                          |
|                                      |              | 1 min.          | 24 hr.                             |                 |                          |
| Tension, 25° C., 15 min.             | 45.9         | 50              | 34                                 | 7.3             | 4.6                      |
| Slack, 25° C., 15 min.               | 43.8         | 60              | 36                                 | 7.3             | 5.2                      |
| Tension, 92° C., 60 min.             | 41.9         | 60              | 37                                 | 6.7             | 4.7                      |
| Slack, 92° C., 60 min.               | 41.6         | 66              | 37                                 | 7.2             | 5.1                      |
| Tension, 92° C., 60 min., NaSCN (7%) | 37.2         | 57              | 34                                 | 5.9             | 3.9                      |
| Slack, 92° C., 60 min., NaSCN (7%)   | 41.4         | 62              | 36                                 | 5.9             | 4.2                      |
| Untreated control                    | 51.5         | 22              | 10                                 | 1.4             | 1.1                      |

treated in 23% sodium hydroxide solution containing 1% Dypenol wetting agent under each of the conditions listed for mercerization. The single yarn properties (as obtained on the Uster Automatic Single Yarn Tester) of the unrelaxed yarns after they had been washed, dried, and backtwisted 15TM in the S direction are shown in Table 3.

## EXAMPLE 4

60

The yarns prepared in Example 3 were woven into fabric using them as filling yarns only with 40 picks per inch filling. The fabric was relaxed in hot water and dried. The stretch properties of these fabrics are shown in Table 4. These fabrics show excellent elongation at break of the 1 inch strips and high stretch values in the 2 inch strips. The recovery from stretch after 24 hours relaxation is good.

We claim:

1. A process for imparting improved stretch properties to a cellulosic yarn comprising
  - (a) wetting a cellulosic yarn of normal-twist or high-twist construction, while said yarn is under no tension or under a tension just sufficient to maintain its length constant, with an aqueous solution containing about 23% by weight of sodium hydroxide and about 1% by weight of a wetting agent compatible with the said 23% sodium hydroxide solution, about from 25° to 92° C. for a period of time of about from 15 to 60 minutes, to swell the yarn;
  - (b) washing, drying, souring, and washing and drying the swollen yarn of step (a);
  - (c) back-twisting the dried yarn of step (b); and

(d) allowing the back-twisted yarn of step (c) to relax in water.

2. The process of claim 1 wherein the cellulosic yarn is of normal-twist construction.

3. The process of claim 1 wherein the cellulosic yarn is 5 of high-twist construction.

4. The process of claim 1 wherein the wetting of the yarn in step (a) is carried out while the yarn is under no tension.

5. The process of claim 1 wherein the wetting of the 10

yarn in step (a) is carried out while the yarn is under a tension just sufficient to maintain its length constant.

#### References Cited

#### UNITED STATES PATENTS

|           |         |                  |       |         |
|-----------|---------|------------------|-------|---------|
| 2,463,618 | 3/1949  | Heberlein et al. | ----- | 57—157  |
| 3,127,732 | 4/1964  | Brown et al.     | ----- | 57—164  |
| 3,285,690 | 11/1966 | Cooper et al.    | ----- | 8—116.3 |

JOHN PETRAKES, *Primary Examiner.*